

# UNITED STATES PATENT OFFICE.

ARTHUR LINZ, OF NEW YORK, N. Y., ASSIGNOR TO THE CHEMICAL FOUNDATION INCORPORATED.

## METHOD OF DYEING.

1,414,030.

Specification of Letters Patent. Patented Apr. 25, 1922.

No Drawing.

Application filed September 1, 1921. Serial No. 497,706.

To all whom it may concern:

Be it known that I, ARTHUR LINZ, a citizen of the United States, and a resident of the borough of Manhattan, city, county, and 5 State of New York, have invented an Improvement in Methods of Dyeing, of which the following is a specification.

My invention relates to an improved method of dyeing and has as an object the 10 obtainment of more permanent and fast to light dyeings upon various materials, whereas such dyeings heretofore have been of a relatively fugitive and unstable character.

When various materials, such as for example, textiles, leather, hides, and so on, are dyed by the ordinary method, the colors are 15 not always permanent and are sometimes affected by the light. It is an object of my improved method to obviate these possible 20 objections and it is shown that when textiles, leather, and so on, are treated in accordance with my method, the colors obtained thereon are relatively faster and more permanent.

The dyeings hereinbefore referred to 25 depend upon the formation of color lakes and the previous processes for producing these lakes upon various materials are not of such a character as to permit of their general adoption, for the reason that these processes 30 are expensive in consequence of the chemicals employed therein, which chemicals may be produced only through the expenditure of considerable time and labor.

The color lake formation upon textiles, 35 and so forth, has been accomplished through the employment of complex acids containing tungsten, such as for instance, phosphotungstic acid and silicotungstic acid or salts of these complex acids. The preparation of 40 the complex acids or the salts thereof with the attendant separation of the same from the by-products, is an involved, difficult and expensive procedure, and accordingly their use has materially affected dyeings dependent upon the formation of the color 45 lakes produced through the intermediation of such complex acids or their salts.

I have discovered a procedure for the dyeing of textiles, leather, and so on, through 50 the formation of color lakes produced through the use of compounds containing phosphorus and silicon, which shall, during the procedure, interact with compounds containing a difficultly fusible metal, which procedure 55 does not involve the production and

isolation of complex acids of difficultly fusible metals or salts of difficultly fusible metals and hence accomplishes a saving of all the expense incident thereto.

Further, in consequence thereof my process 60 presents a mode whereby color lakes may be generally applied in dyeing the various materials and at a cost which will admit of their general use and application.

The process according to my invention, 65 comprises an after treatment of the dyeings of textiles, leather, and so on, with compounds containing phosphorus and silicon together with compounds containing a difficultly fusible metal, of which compounds 70 various ones may be used such as, for instance, the acids, that is phosphoric or silicic or their salts, and compounds of such metals as tungsten or molybdenum, and in accordance therewith it has been ascertained that 75 such dyeings of textiles, leather, and so on, are relatively permanent.

The following example will serve as an 80 illustrative embodiment of a manner in which my process may be carried into practical effect:

### Example I.

Take a quantity of textile, leather, hides, 85 skins or the like, (for example one hundred pounds) mordanted with tannic acid and an antimony salt, or tannin bearing extracts and dye in the usual manner with say about one-half pound of methyl violet. The product has a beautiful purple hue which, however, is fugitive and of a transitory nature. It is then treated by placing in a solution in 90 which has been dissolved a phosphate of sodium, e. g., di-sodium phosphate, and sodium tungstate or a phosphate of sodium 95 and sodium molybdate together with an acid, such as for example, acetic acid, to produce in this solution either sodium phosphotungstate or phospho tungstic acid, or sodium phospho molybdate or phospho 100 molybdic acid. The above salts are added in an amount sufficient to produce about five pounds of the complex salt or its equivalent. The subsequent treatment may be done in the usual manner at ordinary temperature, 105 although it may be considered preferable to carry out the treatment at a raised temperature, about 70° C.

When it is desired to employ salts of an acid of phosphorus or silicon, together with 110

- salts of a difficultly fusible metal, it may be found preferable to add to the dyeing bath a suitable organic or inorganic acid which acid shall be capable of freeing phosphoric, 5 tungstic, molybdic and silicic acids their respective salts, for which purpose there may preferably be used hydrochloric acid, sulphuric acid and acetic acid, which will not effect the coloring matter being used, 10 and it will be understood, of, course, that such acid may be entirely dispensed with if the formation of the color lake takes place satisfactorily without its use, and this may be readily determined by simple treatment.
- 15 The dyestuffs which may be preferably utilized in my process are usually designated as the basic coal tar dyes and in addition to methyl violet set forth in the above example, there may be employed such dyestuffs as 20 auramine, phosphin, chrysoidin, Bismark brown, malachite green, emerald green, methylene blue, Victoria blue, crystal violet, saffranine and basic fuchsin, but it will be understood that my process is not limited to 25 the specific class or the specific dyes herein mentioned, but may be employed for such dyes as will give a permanent and fast color through fixation by means of the compounds set forth.
- 30 I claim:
1. The process of dyeing textiles, leather, and so on, which comprises dyeing the said materials with a basic dyestuff, and then treating said dyed materials with a solution 35 which has been prepared from a soluble compound of tungsten and soluble compound of phosphorus.
  2. The process of dyeing textiles, leather, and so on, which comprises dyeing the said 40 materials, and then treating said dyed materials with a solution which has been prepared from a soluble compound of phosphorus, a soluble compound of tungsten, and an acid capable of freeing the acids of phosphorus and tungsten from their respective salts and which does not affect the coloring matter.
  3. The process of dyeing textiles, leather, and so on, which comprises dyeing the said 45 materials with a basic dyestuff, and then treating said dyed materials with a solution which has been prepared from a soluble compound of phosphorus and a soluble compound of a difficultly fusible metal.
  4. The process of dyeing textiles, leather, 50 and so on, which comprises dyeing the said materials, and then treating said dyed materials with a solution which has been prepared from a compound of phosphorus, a compound of tungsten and an acid capable of freeing the acids of phosphorus and tungsten from their respective salts and which will form a double salt of tungsten in the presence of a coloring matter without destroying said coloring matter.
  5. The process of dyeing textile, leather, 55 and so on, which comprises dyeing the said materials, and then treating said dyed materials with a solution which has been prepared from a phosphate of sodium and a compound of tungsten.
6. The process of dyeing textile, leather, and so on, which comprises dyeing the said materials, with a basic dyestuff, and then treating said dyed materials with a solution which has been prepared from a compound of phosphorus and a tungstate. 70
7. The process of dyeing textile, leather, and so on, which comprises dyeing the said materials, and then treating said dyed materials with a solution which has been prepared from a phosphate of sodium and a tungstate of sodium. 80
8. The process of dyeing textile, leather, and so on, which comprises dyeing the said materials, and then treating said dyed materials with a solution which has been prepared from a compound of tungsten and a di-sodium phosphate. 85
9. The process of dyeing textile, leather, and so on, which comprises dyeing the said materials, and then treating said dyed materials with a solution which has been prepared from a compound of phosphorus and sodium tungstate. 90
10. The process of dyeing textile, leather, and so on, which comprises dyeing the said materials, and then treating said dyed materials with a solution which has been prepared from a sodium tungstate and di-sodium phosphate. 95
11. The process of dyeing textile, leather, and so on, which comprises dyeing the said materials, and then treating said dyed materials with a solution which has been prepared from di-sodium phosphate, sodium tungstate and an acid capable of freeing the acids of phosphorus and tungsten from their respective salts and which will form a double salt of tungsten in the presence of a coloring matter without destroying said coloring matter. 105
12. The process of dyeing textile, leather, and so on, which comprises dyeing the said materials, and then treating said dyed materials with a solution which has been prepared from sodium tungstate, di-sodium phosphate and acetic acid. 110
13. The process of dyeing textile, leather, and so on, which comprises dyeing the said materials, and then treating said dyed materials with a solution which has been prepared from sodium tungstate, di-sodium phosphate and an acid capable of freeing the acids of phosphorus and tungsten from their respective salts. 115
- In testimony whereof, I have signed my name to this specification this 30th day of August, 1921.
- ARTHUR LINZ.